

Patented June 5, 1923.

1,457,375

# UNITED STATES PATENT OFFICE.

VICTOR LOUGHEED, OF SAN FRANCISCO, CALIFORNIA, ASSIGNOR TO ENTERPRISE FOUNDRY COMPANY, OF SAN FRANCISCO, CALIFORNIA, A CORPORATION OF CALIFORNIA.

## MOLD MIXTURE.

No Drawing.

Application filed August 18, 1919. Serial No. 318,209.

*To all whom it may concern:*

Be it known that I, VICTOR LOUGHEED, a citizen of the United States, and a resident of San Francisco, in the county of San Francisco and State of California, have invented certain new and useful Improvements in Mold Mixtures, of which the following is a specification.

In making certain kinds of highly accurate castings, such as dental inlays and small brass or other machine parts, the result is secured by providing a pattern of wax or other similar material cast or molded in a metal or other die, with or without subsequent finishing, and coating and surrounding this pattern with mold or investing material from which, after the mold is hardened or set, the pattern is removed by the expedient of melting, dissolving, or burning out the wax, after which the casting is produced by pouring molten metal into the cavity. It is known that when a very refractory metal is used in this system of casting, the mold material, if a good heat conductor, will chill the metal too rapidly and prevent it from filling the mold completely. In addition to this the desirability has been recognized of having the finished mold of a porous nature so as to vent, more or less freely from its interior, air and gases which, if retained, will form blow-holes and render the finished casting unsound.

When a metal is used for the casting which is highly reactive as to a material of the mold it will tend to attack the mold. The reaction will be particularly favored if the volume of the casting is great so that it remains fluid for a relatively long period of time, and even though it be small, if the heat conductivity of the mold material is so low that in spite of small casting volume the casting remains fluid for a relatively long period of time. Because of these conditions, it is desirable that the mold material be constituted of refractory oxides or other compounds which are not readily reduced at a high temperature in the presence of the molten metal used for the castings. The exclusive use of such constituents, however, introduces difficulties in the way of manufacturing and handling the molds, particularly with respect to the proper binding together of the mold constituents; and these difficulties are hard to overcome by the mere selection of substances that act as a

binder in the first instance. The desired end can be attained, however, if the chemical constitution of the mold can be changed to render it properly coherent subsequent to its first pouring and setting around the pattern, but prior to the pouring of the molten metal.

In the particular case of the use of calcium sulphate as a binder for molds in which copper-containing alloys are to be cast, it is usual to heat the mold in preparation for pouring the metal, in order to first drive off the water of hydration from the calcium sulphate. But unless the temperature reached be excessively high and prolonged, the sulphur trioxide molecule will remain in combination with the calcium oxide molecule, and subsequently be reduced in contact with the hot metal, with the result that the copper of the poured metal will combine with the sulphur and produce, over the surface of the casting, a coating of indigo-blue copper sulphide varying in thickness according to the mass of the individual casting and the time during which it remains molten in contact with the mold material. This coating is exceedingly difficult to remove and seriously impairs the accuracy and finish of the castings.

The object of my invention is to provide a mold composition or mold in which, for convenience of production, calcium sulphate is used as one of the ingredients, but from which this compound is subsequently removed or chemically broken up, and, if necessary, replaced by another binder material. To this end, in addition to the calcium sulphate, kieselguhr, and other ingredients of which the mold may be made, I introduce a proportion of carbon, preferably in the form of finely-powdered wood charcoal, or of metallic aluminum in the form of fine powder, or other ingredient or ingredients, which, when heated, will combine with either the oxygen or the sulfur of the sulfur trioxide molecule to the end of substituting in the mold a compound of sulfur irreducible under the conditions subsequently to be encountered, or also volatile so that it will be dissipated from the mold in gaseous form. I find it desirable, although not absolutely essential, to also introduce a small percentage of kaolin, or china clay, (hydrous aluminum silicate) which will combine with the other materials of the mold at a high tem-

perature, and then act as a binder. It is desirable that the reducing material be present in exactly molecular proportions, or in excess of these, to insure the complete reduction of all of the  $\text{SO}_3$  that is present.

I claim:

1. A porous mold for casting metal, said mold being composed mainly of a refractory porous substance and containing calcium sulphate limited in quantity to that sufficient for binding together the said substance without destroying its porosity, and a basic substance capable of combining with the tri-oxide element of the binder and limited in quantity to that sufficient to render said element non-reactive with respect to the metal to be cast.

2. A porous mold for casting metal composed mainly of a body of refractory porous material together with calcium sulphate limited in quantity to that sufficient to bind

said porous substance and containing carbon in a quantity limited to that sufficient to combine with the oxygen of the calcium sulphate and render the latter non-reactive as to the metal to be cast, but insufficient to impair the porosity of the mold.

3. A mold mixture composed mainly of a refractory porous substance but containing calcium sulphate limited in quantity to that sufficient to act as a binder for said substance without impairing the porosity thereof, and a finely divided basic substance having the capacity to combine with the sulphuric oxide of the binder and render it non-reactive as to the metal to be cast; said basic substance being in finely divided form but insufficient in quantity to impair the porosity of the mold.

Signed at Chicago, Illinois, this 25th day of July, 1919.

VICTOR LOUGHEED.